

Sept 10, 1957

J. E. LAWVER

2,805,770

METHOD OF BENEFICIATING MULTICOMPONENT ORE

Filed Sept. 29, 1953



INVENTOR:  
BY *James E. Lawver,*  
*Ernest V. Haines*

ATTORNEY.

1

2,805,770

**METHOD OF BENEFICIATING  
MULTICOMPONENT ORE**

James E. Lawver, Lakewood, Colo., assignor to International Minerals & Chemical Corporation, a corporation of New York

Application September 29, 1953, Serial No. 382,918

20 Claims. (Cl. 209—127)

This invention relates to an electrostatic method of 15 beneficiating ore materials. More particularly, it relates to the concentration of multicomponent ore materials reducible to an unlocked granular form. Still more particularly it relates to the recovery by electrostatic separation of relatively pure components of nonmetallic materials such as phosphate, silica, sylvite, feldspar, fluorspar, and the like.

Electrostatic beneficiation of minerals has been practiced in a number of forms. It has been commonly utilized to separate conductors from nonconductors. Apparatus utilizing corona discharge, or using a rotating roll, which is one of a pair of electrodes, are examples of equipment for this type of operation. A second system utilizable for separation of conductors from conductors and nonconductors from nonconductors has been the selective reagentizing of materials so that they may be processed as though the separation were one of removing conductors from nonconductors. Electrostatic separation has been applied in still a third form to separate nonconductors. In the latter system, the nonconductors are selectively induced to accept a positive or a negative charge and then are separated as freely-falling bodies drawn in the direction of one or the other of the electrodes being maintained at a high impressed difference of potential.

When separating nonconductors by the last outlined system, many mineral ores, after concentration to a greater or lesser degree, exhibit weak or incomplete charging as proven by the reaching of a stage wherein the ore particles, or some components thereof, show little or no tendency for movement in response to an electrostatic field. Treatment of such ore concentrates in the manner initially utilized to induce charging, such as by contacting a grounded donor plate, or introducing thermal energy and the like, as well as combinations thereof, have failed to render the concentrates sufficiently responsive to an electrostatic field to effect recovery of concentrates of the desired higher component content.

It is a primary object of the instant invention to provide a process for the recovery of concentrates of a high degree of purity.

It is a further object of the instant invention to provide a process wherein the use of reagents such as are commonly employed in flotation processes is eliminated.

It is still a further object to provide a method whereby electrically inactive ore concentrates are again rendered responsive to an electrostatic field.

It is a further object of the instant invention to provide a simplified separation method for nonmetallic ore material.

It is a still further object to provide a process wherein charged coarse grains of a material capable of exchanging electrons through contact potential means with the components of a concentrate is recirculated to improve the charging of ore particles, and is then removed by methods other than electrostatic separation.

2

These and other objects of the novel method will be more fully understood from the following description.

The method of the instant invention is based upon the discovery that ore concentrates which exhibit poor 5 charging characteristics and, therefore, are not subject to any appreciable upgrading by subsequent passes through electrostatic fields may be caused to charge to an extent restoring response to electrostatic fields by tribo-electrification in the presence of a mechanically removable 10 material of work function different from the ore component exhibiting the insufficient charging for electrostatic field response.

By the terminology "work function different from the ore component" is meant the characteristic of exchanging electrons with the ore component whereby the ore component exhibits a definite charge. Materials which receive electrons are generally referred to as having a higher work function than the donor material. Applicant does not wish to be bound by theory, but includes 20 equivalent applications by which ore components exhibiting insufficient charge for effecting separation are, by contact with a removable material, caused to show a response to electrostatic fields warranting additional passes for further ore concentration.

25 In carrying out this novel method, the nonconductor material of work function different from the ore component to be concentrated and separable from the ore by means of differences of shape, differences in size, specific gravity, or other utilizable distinguishing characteristics, 30 is mixed with said ore concentrate which initially or subsequently shows substantially no response to electrostatic separation. The mixture of ore and coarse nonconductor material is agitated either in the presence of or in the absence of an electrostatic field and the further 35 concentration thereof effected before or after separation of the added coarse granular material.

As applied to the electrostatic beneficiation of phosphate ores, the process involves mixing into either a phosphate concentrate, a silica tail concentrate or other 40 fraction a predetermined quantity of the minor component of the fraction having a size appreciably larger than the largest particles of the material being subjected to electrostatic beneficiation. In the case of phosphate concentrates, granular silica is added to an electrostatically prepared phosphate concentrate and the mixture agitated thoroughly in a dry state to induce the particles 45 selectively to be electrically charged by tribo-electrification. In the case of electrostatically prepared middling 50 fractions from an electrostatic phosphate concentration operation; the addition agent may be either phosphate pebbles or hard rock phosphate of a proper size. When electrostatically treating potash ore such as sylvite, coarse granular halite crystals would be mixed with sylvite 55 concentrates.

In the preferred embodiment, the phosphate ore concentrate and coarse silica are agitated in a mixer whose material of construction has a work function different from either the phosphate or the silica. The charged 60 mixture is screened to effect separation of silica upon a particle size basis. The phosphate ore concentrate is then passed through additional electrostatic separations to obtain a phosphate product of high purity.

65 When the process is placed on a continuous basis, the method of beneficiating phosphatic ore comprises mixing dry concentrate with a predetermined amount of a recycle stream of coarse silica of an average particle size larger than the largest particles of concentrate, electrostatically separating the mixture, recovering at least a 70 concentrate portion and a tailing portion, and screening the coarse silica from appropriate fractions for recycle

to the system; if such screening is not made before the electrostatic separation.

In the preliminary treatment of ores prior to any passage through electrostatic fields, the ore is treated so as to have a reasonable uniform particle size. In the case of Florida phosphate pebble ore, the operation is purely one of washing to free the phosphate pebbles of matrix and then sizing to produce a fraction in the range of about 14 mesh to about 200 mesh. Only Florida phosphate pebbles of +14 mesh size are subjected to any grinding operation in the preparation of feeds which are to be subjected to beneficiation treatments. On the other hand, phosphate ores from other regions, and other non-conductor mineral ores, require grinding to the economic liberation stage for freeing or unlocking the undesired ore components. Different types of material being fed to an electrostatic field will have different particle sizes, but in general the particle size will fall in a range between about 14 mesh and about 325 mesh. Some of the different types of materials having a somewhat shorter range of particle size as, for example, washer debris, phosphate, or fines, have a particle size in the range between about 14 mesh and about 150 mesh whereas, the fines from low-grade pebble grinding operations often have a particle size in the range of about 150 mesh to about 325 mesh.

The multicomponent material, freed as individual particles, is next dried. This may be accomplished either by direct or indirect heating; for example, by contacting a bed of granular material with hot gases, as in a rotary kiln, tunnel dryer, electric oven, or the like. In the dryer the solids are raised to an elevated temperature, the temperature for such ores as sylvinitic being in excess of about 675° F. the temperature being that which conditions the ore for charging and separation, while ores such as phosphate need only be raised to a temperature in excess of the optimum for separation. After heating, the ore is induced selectively to accept an electrical charge, either during the cooling down period or after cooling to the optimum temperature for separation, by such contact potential methods as strong agitation under particle to particle contact conditions or so-called tribo-electrification or by particle to donor element contact with or without the donor being grounded to the earth.

Charged material is fed as freely-falling bodies between electrodes held at a high difference of potential. After one or more electrostatic separations, the ore concentrates begin to exhibit an appreciable reduction in response to the forces acting in an electrostatic field even though they still are maintained at an elevated temperature and are subjected to donor element contact. When this stage of concentration is reached, the particles are treated in accordance with this invention in order to make them again approach their initial activity. Phosphate concentrates, for example, which have become inactive, are then mixed with coarse silica having a particle size in the range between about 4 mesh and about 10 mesh, the preferred silica material being relatively uniform in size. The recharging of the ore concentrate-added component of different work function mixture may then be accomplished by intimately contacting one another in a suitable mixer. By intimate contact, the particles exchange electrons and thereby materials of different nature acquire either a positive or a negative charge. Recharging is preferably carried out in a suitable mixer, such as a rotating cylinder, a paddle mixer, or the like, partially or wholly of metal construction, such as iron, steel, copper, copper alloys, and the like.

Mixtures of materials respond differently depending upon the relative work functions of the materials of the concentrate and the added component of different work function, and therefore, generalizations applicable in all situations are difficult to set forth. A material may be of such nature as to impart to phosphate a charge of greater

or lesser magnitude than silica. It is believed sufficient to state, therefore, that combinations of ingredients or ingredients plus material of the mixer where the mixer may act as a donor element should result in the charging of the concentrate material whereby particles of one kind are given a charge and particles of another type acquire a charge of different character or different magnitude such that they may be effectively separated by passage through an electrostatic separating unit.

In the preferred embodiment, after intimate contacting, the added material is segregated by screening. The now charged concentrate is next subjected to one or more passes through electrostatic fields as freely-falling bodies, i. e., in a path normally not in contact with the electrodes. In both the initial stages of separation and the final stages of separation, the strength of the electrostatic field which will effectively alter the path of particle movement varies with the average particle size of the feed to the separator unit. The field gradient in such operations may vary from 3,000 volts per inch of distance between electrodes in separating material of relatively fine particle size to 15,000 volts per inch of distance separating electrodes for beneficiation of coarser particles. In all such discussion of field strength, it must be borne in mind that corona discharges which ionize air are to be avoided. In general, it is preferred to operate at a total impressed difference of potential in the range of about 50,000 volts to about 250,000 volts. This voltage should be maintained at a high direct voltage potential substantially free of alternating current components, i. e., filtered D. C. current should be low in the so-called A. C. ripple. A steady and relatively inexpensive supply of D. C. voltage may also be obtained by the use of such equipment as radio frequency power supply.

The invention will be more fully understood from the following description taken in conjunction with the attached flow sheet, it being understood that the foregoing flow sheet illustrates but one method of taking advantage of the invention, i. e., processing of phosphate concentrate, and that other equivalent methods will be obvious, i. e., processing of desired component fractions, such as tail fractions, middling fractions, etc.

Referring to the flow sheet for phosphate beneficiation, ore of a mesh size in the range between about 14 mesh and about 200 mesh passes from storage bin 19 to a heating station 11 where the ore material is raised to a temperature in the range between about 200° F. and about 350° F. or even up to about 500° F. Preferably while still hot, the dried material is conveyed to a charging station 12 where the particles are induced to take on an electrical charge, as by passage over a grounded contact surface of graphite, lead, zinc, aluminum, copper, tin, and the like. The charged feed is next delivered to an electrostatic separation unit 13 which may consist of one or more stages of electrostatic separation. At separation unit 13 there is produced a throw-away tail fraction 14 and an intermediate concentrate 15. The intermediate concentrate 15 is commingled with coarse material, such as silica, of a particle size appreciably larger than that of the largest particle of the concentrate at the mixer-electron recharging station 16. The mixed and charged material issuing from station 16 in the preferred embodiment of the invention is conveyed to screening station 17 where the coarse material, such as silica, is removed. The said coarse material is returned by conveyor 18 to coarse material storage 19 pending recycling to the mixer-recharging station 16. The charged concentrate is then passed with or without reheating to an electrostatic separation unit 20. Upon passage through one or more stages of electrostatic separation, at least two products, and usually three products, are collected; namely, a final concentrate fraction 21, a middling fraction 22, which generally is recycled to recover a component therefrom, and a tail fraction 23.

In an alternative mode of operation, the intermediate concentrate 15 is commingled with coarse material, such as silica, of a particle size appreciably larger than that of the concentrate at the mixer-charging station 16. The mixed and charged material issuing from station 16 is moved by conveyor 25 to electrostatic separation unit 20. Upon passage through one or more stages of electrostatic separation, at least two products, and usually three products are collected; namely, a predominantly concentrate fraction 21, a middling fraction 22, and a predominantly tail component fraction 23. Each of these fractions, or only some, may be conveyed to a screening station 26, depending upon the nature of the coarse material where the coarse material may be separated, if desired. If the coarse material is to be recycled, it is returned to storage station 19 by conveyor 27. Materials which may be either concentrate or tail, or both, collected individually, are segregated for storage or for further processing.

The following examples are given to illustrate an application of the instant novel process to Florida phosphate rock and to sylvinitic ore and are not to be construed as limiting the invention thereto.

*Example I*

Florida phosphate ore was washed to produce a low-grade Florida phosphate pebble ore having a B. P. L. content of approximately 30%. The pebble material had a particle size in the range of about 14 and about 200 mesh. This material was dried at a temperature of approximately 225° F. The pebble material was passed while hot through four stages of electrostatic separation at which time a concentrate was produced constituting approximately 20% by weight of the feed and having approximately 73.5% B. P. L. content and approximately 8% of insoluble material. These separations were each effected by passage of feed material at a rate of approximately one ton per hour per linear foot of electrode between 10 feet long electrodes spaced approximately 9 inches apart and having a difference of potential impressed thereon such that the field gradient was approximately 10,000 volts per inch of distance separating the electrodes.

The intermediate concentrate was segregated into two portions for comparative tests. Upon passage of the first portion through a fifth stage of electrostatic separation under identical electrostatic conditions as was maintained previously, a concentrate and tail was produced of substantially identical analyses showing that no effective separation was being accomplished.

The second portion of the intermediate concentrate was mixed with 20% by weight of coarse silica of a particle size of about +10 mesh. The mixture was then agitated in an iron paddle mixer allowing the mixture a retention period of about twenty minutes. The coarse silica was recovered by seiving the mixture on a 10 mesh Tyler standard screen. The concentrate passing through the screen was delivered at a rate of approximately one ton per hour per linear foot of electrode through a fifth stage of electrostatic separation. The concentrate recovered had approximately 78% B. P. L. content and approximately 2.5% of insoluble material. This concentrate constituted a recovery of approximately 70% of the original phosphate content as premium grade pebble material. The middling phosphate stream which was to be recycled accounted for approximately 17% of the phosphate content of the original phosphate pebble material. A comparison of the results is as follows:

|                               | Concentrate                 |                     | Tail,<br>Percent<br>B. P. L. |
|-------------------------------|-----------------------------|---------------------|------------------------------|
|                               | Percent<br>B. P. L.<br>Feed | Percent<br>B. P. L. |                              |
| Untreated Material.....       | 73                          | 73                  | 73.0                         |
| Mixer Recharged Material..... | 73                          | 78                  | 70.0                         |

As can be seen from the above comparison, the separation effected in the fifth stage produces a premium grade phosphate and, by a recycling system for the high B. P. L. content tail, an approximately 85% recovery of the phosphate can be effected as this high-grade product.

*Example II*

Slime-bearing sylvinitic ore from the Carlsbad section of New Mexico was crushed and then comminuted in a hammer mill.

- 10 The comminuted ore was screened to produce a fraction containing particles in the range between about 14 mesh and about 200 mesh size. This granular sylvinitic feed was heated to approximately 800° F. Heating when the solids attained this temperature, was continued for about five minutes. The material was then removed from the heating unit and cooled to approximately 375° F. The particles were delivered to a feed hopper and cascaded downwardly through a vibratory cast-iron trough. The granular material differentially charged, halite charged positively, and sylvite charged negatively, cooled to about 225° F. during delivery and was allowed to drop between vertical electrodes at a rate of approximately 2000 pounds per hour per foot of horizontal electrode breadth. The electrodes had a difference of potential of approximately 100,000 volts impressed thereon giving a field gradient of approximately 10,000 volts per inch of distance between oppositely charged electrodes. In the first pass through the electrodes, a concentrate was recovered. This concentrate was split into two portions.
- 15 20 25 30 35 40 45 The first portion was reheated for one hour in an oven held at approximately 800° F. This reheated portion was screened to remove +28 mesh size material and then was passed through an electrostatic unit identical to that used for the first or rougher separation.
- 35 The second portion of this sylvite concentrate was mixed with halite crystalline material of a particle size of about 14 mesh. This mixture containing a 2 to 1 ratio by weight of second portion of the concentrate and added halite was heated to 800° F. in the same manner as the first portion of the concentrate. The reheated mixture during cooling was agitated in a stirring mixer. The agitated mixture was then screened to remove the added material and then was passed through the same electrostatic unit as was used for separation of the first portion of the concentrate.

45 The assay of the various concentrates shows that addition of coarse halite to the sylvinitic rougher concentrate improves the separation. These assays are as follows:

| 50                                            | Feed,<br>Percent<br>K <sub>2</sub> O | Concen-<br>trate,<br>Percent<br>K <sub>2</sub> O | Tail,<br>Percent<br>K <sub>2</sub> O |
|-----------------------------------------------|--------------------------------------|--------------------------------------------------|--------------------------------------|
| Untreated sylvinitic rougher concentrate..... | 35                                   | 51                                               | 15                                   |
| Mixer recharged concentrate.....              | 35                                   | 53                                               | 13                                   |

55 In each case the recovery of KC1 in the final concentrate was 55% of the weight of sylvite in the rougher concentrate used as feed material to the last separation.

This application is a continuation-in-part of application 60 Serial No. 222,690, filed April 24, 1951, now abandoned.

Having thus fully described and illustrated the character of the invention, what is desired to be secured and claimed by Letters Patent is:

- 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 881

to at least one electrostatic separation, mixing with the concentrate produced by said separations a predetermined quantity of solid particles of material of work function different from the mineral component being concentrated and agitating the mixture whereby the concentrate is induced selectively to accept an electrical charge, and subjecting the charged ore concentrate material to additional electrostatic separation.

3. A method of beneficiating ore which comprises subjecting a multicomponent nonconductor mineral ore feed to at least one electrostatic separation, adding to the concentrate produced a predetermined quantity of solid particles of material of work function different from the mineral component being concentrated, agitating the mixture under conditions to effect tribo-electrification, and subjecting the charged ore concentrate material to electrostatic separation.

4. A method of beneficiating ore which comprises subjecting a nonconductor mineral ore feed to at least one electrostatic separation, mixing with the concentrate produced a predetermined quantity of solid particles of material of work function different from the mineral component being concentrated and agitating the mixture whereby the concentrate is induced selectively to accept an electrical charge, separating the added material from the ore concentrate, and subjecting the charged ore concentrate material to additional electrostatic separation.

5. A method of beneficiating ore which comprises subjecting a nonconductor mineral ore feed to at least one electrostatic separation, mixing with the concentrate produced a predetermined quantity of solid particles of material of work functions different from the mineral component being concentrated whereby the concentrate is induced selectively to accept an electrical charge, segregating the added material by mechanical means, and subjecting the charged concentrate to the attractive and repulsive forces of one or more electrostatic fields.

6. A method of beneficiating ore which comprises subjecting a nonconductor mineral ore feed having a particle size range between about 14 mesh and about 325 mesh to at least one electrostatic separation, mixing with the concentrate produced by said separations a predetermined quantity of solid particles of material of work function different from the mineral component being concentrated having a particle size larger than the largest particle of the ore feed and agitating the mixture whereby the concentrate is induced selectively to accept an electrical charge, and subjecting the charged ore concentrate material to additional electrostatic separation.

7. A method of beneficiating ore which comprises subjecting a nonconductor mineral ore feed having a particle size range of between about 14 mesh and about 200 mesh to at least one electrostatic separation, mixing with the concentrate produced a predetermined quantity of solid particles of material of work function different from the mineral component being concentrated and having a particle size range between about 4 mesh and about 10 mesh, and subjecting the charged ore concentrate material to further electrostatic separation.

8. A method of beneficiating ore which comprises subjecting a nonconductor mineral ore feed having a particle size range between about 14 mesh and about 200 mesh to at least one electrostatic separation, mixing with the concentrate produced a predetermined quantity of solid particles of material having a particle size range between about 4 mesh and about 10 mesh and of work function different from the mineral component being concentrated, screening the mixture to recover the material having a particle size range between about 4 mesh and about 10 mesh, and subjecting the charged ore concentrate material to further electrostatic separation.

9. A method of beneficiating ore which comprises subjecting a nonconductor mineral ore feed having a particle size in the range between about 14 mesh and about 200 mesh to at least one electrostatic separation,

mixing with the concentrate produced a predetermined quantity of solid particles of material of work function different from the mineral component being concentrated and having a particle size in the range between about 4 mesh and about 10 mesh, screening the mixture to recover the material having a particle size between about 4 mesh and about 10 mesh, subjecting the charged ore concentrate material to electrostatic separations as freely-falling bodies, and collecting at least a concentrate fraction and a tail fraction in the vicinity of the lower portions of the electrodes bounding said electrostatic field.

10. A process as in claim 9 wherein the concentrate fraction is screened to recover the beneficiated ore fraction.

11. A method of beneficiating ore which comprises subjecting a relatively uniform particle size nonconductor mineral ore feed to at least one electrostatic separation in an electrostatic field having a field gradient in the range between about 3,000 volts per inch and about 15,000 volts per inch of distance separating electrodes, mixing with the concentrate produced by said separations a predetermined quantity of solid particles of material of different physical characteristics and of work function different from the mineral component being concentrated whereby the concentrate is induced selectively to accept an electrical charge, and subjecting the charged ore concentrate material to additional electrostatic separation.

12. A method of beneficiating phosphate ore which comprises subjecting a raw phosphate feed having a particle size range between about 14 mesh and about 200 mesh to at least one electrostatic separation, adding to the concentrate produced silica having a particle size range between about 4 and about 10 mesh, agitating the mixture under conditions to effect tribo-electrification, screening the coarse silica from the agitated mixture, and subjecting the charged phosphate material to further electrostatic separation.

13. A method of beneficiating potash ore which comprises subjecting potash ore having a particle size range between about 14 mesh and about 200 mesh to at least one electrostatic separation, adding to the concentrate produced halite material having a particle size larger than about 14 mesh, agitating the mixture under conditions to effect tribo-electrification, screening the coarse halite material from the agitated mixture, and subjecting the charged potash concentrate to further electrostatic separation.

14. A method of beneficiating electrostatically prepared ore concentrates which exhibit substantially no response to an electrostatic field due to loss of charge during electrostatic separation which comprises mixing with said concentrate a predetermined quantity of solid particles of material of work function different from the mineral component being concentrated whereby the concentrate is induced selectively to accept an electrical charge, and subjecting the charged ore concentrate material to additional electrostatic separation.

15. A method of beneficiating electrostatically prepared ore concentrates which exhibit substantially no response to an electrostatic field due to loss of charge during electrostatic separation which comprises adding to the concentrate a predetermined quantity of solid particles of material of work function different from the mineral component being concentrated, agitating the mixture under conditions to effect tribo-electrification, and subjecting the charged ore concentrate material to electrostatic separation.

16. A method of beneficiating electrostatically prepared ore concentrates which exhibit substantially no response to an electrostatic field due to loss of charge during electrostatic separation which comprises mixing with the concentrate a predetermined quantity of solid particles of material of work function different from the mineral component being concentrated whereby the concentrate is induced selectively to accept an electrical charge, segregating the added material by mechanical

means, and subjecting the charged concentrate to the attractive and repulsive forces of one or more electrostatic fields.

17. A method of beneficiating electrostatically prepared ore concentrates having a particle size range of between about 14 mesh and about 200 mesh which exhibit substantially no response to an electrostatic field due to loss of charges during electrostatic separations which comprises mixing with the concentrate a predetermined quantity of solid particles of material of work function different from the mineral component being concentrated and having a particle size range between about 4 mesh and about 10 mesh, and subjecting the charged ore concentrate material to further electrostatic separation.

18. A method of beneficiating electrostatically prepared ore concentrates which exhibit substantially no response to an electrostatic field due to loss of charges during electrostatic separation which comprises mixing with the concentrate a predetermined quantity of solid particles of material of work function different from the mineral component being concentrated and agitating the mixture whereby the concentrate is induced selectively to accept an electrical charge, and subjecting the charged ore concentrate material to additional electrostatic separation in an electrostatic field having a field gradient in the range between about 3,000 volts per inch and about 15,000 volts per inch of distance separating electrodes.

19. A method of beneficiating electrostatically prepared ore concentrates having a particle size in the range between about 14 mesh and about 200 mesh and which exhibit substantially no response to an electrostatic field due to loss of charges during electrostatic separation which comprises mixing with the concentrate a predetermined quantity of solid particles of material

of work function different from the mineral component being concentrated, screening the mixture to recover the nonconductor material having a particle size range between about 4 mesh and about 10 mesh, and subjecting the charged ore concentrate material to at least one electrostatic separation as freely-falling bodies, and collecting at least a concentrate fraction and a tail fraction in the vicinity of the lower portions of the electrodes bounding said electrostatic field.

10 20. A method of beneficiating electrostatically prepared Florida phosphate ore concentrates having a particle size range between about 14 mesh and about 200 mesh and which exhibit substantially no response to an electrostatic field due to loss of charges during electrostatic separation which comprises adding to the concentrate silica having a particle size range between about 4 mesh and about 10 mesh, agitating the mixture under conditions to effect tribo-electrification screening the coarse silica from the agitated mixture, and subjecting the charged ore concentrate material to further electrostatic separation.

#### References Cited in the file of this patent

##### UNITED STATES PATENTS

25 754,756 Edison ----- Mar. 15, 1904  
2,197,865 Johnson ----- Apr. 23, 1940

##### OTHER REFERENCES

30 "Science," vol. 102, #2658, December 7, 1945, pages 575, 576 only of article by Loeb, "The Basic Mechanisms of Static Electrification."

"Industrial and Engineering Chemistry," vol. 32 (1940), article by Fraas and Ralston, "Electrostatic Separation of Solids," pages 600-604.

35 Copies in Scientific Library.